

## UNITED STATES PATENT OFFICE

1,952,083

## ALLOY

Robert H. Leach, Fairfield, Conn., assignor to  
Handy & Harman, New York, N. Y., a corpora-  
tion of New York

No Drawing. Application June 10, 1932.  
Serial No. 616,500

2 Claims. (Cl. 75—1)

This invention relates to silver alloys and is concerned more particularly with a novel silver alloy which may be used to especial advantage in the manufacture of table silver and hollow ware and for various other purposes, because it has the property of strongly resisting tarnish and discoloration.

As is well known, silver alloys of ordinary composition and containing copper as the base ingredient are susceptible to tarnish. Such discoloration of the metal is brought about by numerous agents, the most active being sulphur, which is present in various foods such as eggs, and it is also present to some extent in the atmosphere in the form of gaseous compounds. Sulphur in both forms causes tarnishing at a rate which depends on the length of contact or exposure of the metal, the concentration of the sulphur in the food or air, and the form in which the sulphur is present. In any event, the necessity of frequent cleaning and polishing of silver articles to keep them in bright condition has led to numerous attempts in the past to produce silver alloys which are of good appearance, have the desired working characteristics, and have a better resistance to tarnish than ordinary silver-copper alloys, but up to the present, the proposed alloys with which I am familiar, have not proven entirely satisfactory.

The problem of producing a silver alloy which is resistant to tarnish is a difficult one because investigation has shown that binary alloys offer little promise and the number of ternary and quaternary alloys is very large. When it is understood that small variations in the ingredients in these alloys have an important effect on the resistance to tarnish and the amounts of the alloying ingredients used is highly critical with respect to tarnish resistance, the magnitude and difficulty of the problem will be appreciated.

As a result of my investigations in this field, I have found that a silver alloy which has excellent resistance to tarnish produced by various agents may be made by using tin and magnesium as alloying metals, provided these ingredients are confined within relatively narrow limits. In addition to the tin and magnesium, the new alloy also contains a small amount of a fourth ingredient which not only adds to its tarnish resistance but improves its physical properties. The fourth ingredient may be one or both of the metals, chromium and antimony, and I shall refer to this ingredient as a "hardener", although the hardening effect depends considerably on the amount of the ingredient present and an

amount which increases the tarnish resistance may have little hardening action.

A silver alloy of sterling fineness, made in accordance with the invention, contains not less than about 92.5% silver, tin ranging from about 4% to about 6.5%, magnesium ranging from about 0.5% to about 3%, and one or both of the metals chromium and antimony as hardening elements with these metals present in a total amount ranging from about 0.25% to not substantially in excess of 1.5%.

A typical example of the new alloy of sterling fineness has the following approximate analysis:

|           | Per cent | 70 |
|-----------|----------|----|
| Silver    | 92.5     |    |
| Tin       | 5.5      |    |
| Magnesium | 1.5      |    |
| Chromium  | 0.5      |    |

The new alloy is highly resistant to tarnish and corrosion and it may be given the desired physical characteristics by the addition of the hardening elements in proper amounts. I prefer to use chromium for this purpose and ordinarily it is not necessary to employ more than 0.5% of this metal. The use of chromium in such an amount makes the alloy sufficiently hard for ordinary purposes and the hardness may be increased by increasing the amount of chromium. Antimony also acts as a hardening agent but its effect is less pronounced than chromium. Both chromium and antimony in the amounts specified increase the resistance of the alloy to tarnish and are substantially equivalent for the purpose mentioned.

What I claim:

1. A silver alloy which consists of about 92.5% silver, tin ranging from about 4% to about 6.5%, magnesium ranging from about 0.5% to about 3%, and chromium ranging from about 0.25% to about 1.5%.

2. A silver alloy which consists of about 92.5% silver, about 5.5% tin, about 1.5% magnesium, and about 0.5% chromium.

ROBERT H. LEACH. 100

105

110